

# UNITED STATES PATENT OFFICE.

WILLIAM SYDNEY STEVENS, OF MAGDALENA, NEW MEXICO, ASSIGNOR, BY MESNE ASSIGNMENTS, TO THE OZARK SMELTING AND MINING COMPANY, OF CLEVELAND, OHIO, A CORPORATION OF OHIO.

## METHOD OF CONCENTRATING ORES.

1,116,642.

Specification of Letters Patent. Patented Nov. 10, 1914.

No Drawing.

Application filed December 10, 1912. Serial No. 735,939.

*To all whom it may concern:*

Be it known that I, WILLIAM SYDNEY STEVENS, a subject of the King of Great Britain, and a resident of Magdalena, county of Socorro, and State of New Mexico, have invented a new and useful Improvement in Methods of Concentrating Ores, of which the following is a specification, the principle of the invention being herein explained and the best mode in which I have contemplated applying that principle, so as to distinguish it from other inventions.

The present invention relates generally to the concentration of ores to obtain the valuable constituents, and its particular design is the separation of desired metalliferous sulfids from the associate gangue or from other sulfids. If an ore containing metalliferous sulfids be crushed and mixed with water, certain fatty substances added to the mixture will exhibit a peculiar preferential affinity for the sulfid particles as compared with the gangue-particles, and several processes of ore concentration dependent upon this peculiarity have been proposed.

It has been proposed to concentrate ores by adding to the ore pulp in water a very large quantity of a substance which will exhibit this peculiarity, the quantity added being sufficient to entrap and float upwardly through the water the sulfid particles. Such a process, however, is not effective at all in the concentration of certain ores, and, moreover, it is obvious that in such a process

a very large quantity of the entrapping substance must be used, and it is found in practice that the quantity is prohibitive of the successful working of the process. It has also been proposed to concentrate ores by what may be termed a "frothing process" in which some substance exhibiting a preferential affinity for sulfid particles is added to the ore pulp, after which there are generated in the pulp gaseous bubbles that attach themselves to the sulfid particles and raise them to the surface of a containing body of water (perhaps slightly acidified) in the form of a froth; but both proposal and practice in regard to a frothing process is to use oleic acid or an analogous fatty substance for preferential adherence to the sulfid particles, for a frothing process is only successful when a substance of that nature is employed. It has also been proposed to con-

centrate ores by adding oleic acid, or an analogous fatty substance, to an ore pulp and effecting a flotation of the sulfid particles by the phenomenon of surface tension.

I have attempted to concentrate certain sulfid ores by the various processes known to me and have found that no one of them can be successfully employed in the treatment of those ores. I have ascertained, by thorough experiment with the ores referred to, that in order to effect a separation of the sulfid particles by flotation, whether by frothing or by surface tension, it is necessary to add to the pulp sulfuric acid in order to render any oily substance that may be added effective in preferentially adhering to the sulfid particles. My experiments, however, have resulted in the ascertainment that with the sulfid ores referred to the use of oleic acid or analogous fatty substances to preferentially adhere to the sulfid particles necessitates the consumption, during the process, of such a very large quantity of sulfuric acid that the process becomes impracticable, and this is especially true when the ore to be concentrated is contaminated with carbonates which are easily attacked by the acid. I have also ascertained by experiments that in treating certain sulfid ores if oleic acid or analogous fatty substance be used it acts upon some oxids, such as the specular oxid of iron, equally with the desired sulfid, so that concentration is rendered impossible.

I have ascertained by thorough experiments that certain sulfid ores may be concentrated by a flotation method by using, in conjunction with sulfuric acid, a mineral oil which adheres to the desired sulfid particles while it will not adhere to the undesired particles, and by the use of the process herein described marked separations have been made between the desired sulfid and a gangue including hydrous or anhydrous oxids of iron, iron pyrites, or even other undesired sulfids. It is to be understood that the amounts of mineral oil and acid added to the pulp are to be determined, within certain limits, by experiment. In the treatment of the certain sulfid ores referred to with a mineral oil and sulfuric acid, the amount of acid necessary to a successful concentration is less than one-half the amount necessary if the ore is treated with oleic

acid, or an analogous fatty substance, in place of the mineral oil. I have furthermore ascertained that certain sulfid ores which cannot be concentrated at all by the use of oleic acid, or analogous fatty substance, may be concentrated with entire success by treatment with a mineral oil in conjunction with sulfuric acid.

In the concentration of ores, according to the present invention, the ore is crushed to a suitable degree of fineness, preferably substantially to a powder, and is mixed with sufficient water to form a pulp which will flow fairly freely. A mineral oil is added to the pulp, and I have ascertained that a successful separation of the sulfid particles can be effected by using as a mineral oil what is commonly known as Texas fuel oil, though other petroleum oils of comparatively high boiling-point may also be used with success. The amount of mineral oil added to the pulp is dependent upon the mineralization of the ore under treatment and upon what sulfids it is desired to separate from the ore, but it is to be observed that the amount of mineral oil should only be sufficient to cover the desired sulfid particles with a thin film, and should not be sufficient to agglomerate or entrap and raise the sulfid particles. I have ascertained that in the treatment of the sulfid ores, the concentration of which I particularly desire to effect, the amount of mineral oil required is not over one per cent. of the ore by weight, and generally ranges from three-tenths per cent. to six-tenths per cent. of the ore by weight. Sulfuric acid is also added to the pulp, for its presence permits the action of the mineral oil in selectively coating the desired metalliferous sulfid particles, by decomposing the carbonates which contaminate the ores referred to, and also by cleaning off the sulfid and exposing it to the action of the mineral oil. Sulfuric acid is the only satisfactory acid for this purpose, and I have ascertained, in the treatment of the sulfid ores referred to, that, when a mineral oil is employed for the purpose of coating the sulfid particles, the amount of sulfuric acid need not exceed five per cent. of the ore by weight, and it generally ranges from two per cent. to four per cent. of the ore by weight. The crushed ore and water and mineral oil and acid are now thoroughly mixed in any suitable apparatus.

It is to be understood that the mixing operation is for the purpose of thoroughly presenting the desired sulfid particles to the mineral oil, and is not designed to in any way aerate the mass, and any air bubbles that are produced in the mass by the mixing operation are subsequently broken before the pulp is presented to a liquid surface. I have also ascertained, by thorough experiments, that the rapidity of the mixing oper-

ation is greatly increased, and the action of the mineral oil in selectively coating the metalliferous sulfid particles is rendered possible, by having the mixing take place in a temperature of approximately 70° C., though the temperature may possibly range from 60° C. to 80° C. The high heat is necessary to effect decomposition of the carbonates by the acid, and, among other functions, causes increased activity of the acid in cleaning the sulfid particles and causes increased activity of the mineral oil in selectively coating the sulfid particles. Heat may be applied to the mixture directly, or by heating the water or mineral oil or acid or ore, or any of them, before adding them to the other ingredients.

After the crushed ore, water, mineral oil, and acid, have been thoroughly mixed, at the increased temperature referred to, the flowing pulp is exposed to the air and then presented to the surface of a body of liquid. Any desired apparatus for presenting the pulp to the surface of a liquid may be employed, but it should be such as to break up any air bubbles in the pulp before the latter meets the liquid surface. When the pulp meets the surface of the liquid, the desired metalliferous sulfid particles being coated with a thin film of mineral oil and having been first exposed to air are caused to float on the surface of the water by the phenomenon of surface tension, for the oiled particles do not overcome the tension at the surface of the water, and float. The unoiled particles become wet by the water so that they overcome the tension at the surface thereof, and will not float upon the surface. The separated metalliferous particles and gangue may be collected in any suitable manner. The gangue residue may perhaps still contain some valuable constituents, and these may be recovered by leading the residue to a second mixing apparatus and, if necessary, adding more mineral oil and acid, and then again presenting the mass to a flotation apparatus.

In some ores the desired metalliferous sulfid is contaminated with such large quantities of carbonates or clayey matter that they cannot be successfully concentrated by a flotation process. Such ores may be successfully treated by preliminarily washing them in a suitable apparatus, or by simultaneously tabling and washing the ore, which will remove sufficient of the contaminating matter so that they may be thereafter successfully concentrated by my process.

Certain ores contain, in association with blende or zinc sulfid, a considerable amount of iron pyrites, and such an ore cannot be concentrated by a flotation process because the iron pyrites becomes oiled equally with the blende. Such an ore, however, can be successfully concentrated to secure the blende.

by first roasting it to a sufficient intensity to superficially oxidize the iron pyrites while not sufficiently to materially affect the blende so that in the subsequent treatment with a mineral oil and sulfuric acid the blende becomes oiled while the iron pyrites does not, and upon a subsequent presentation of the pulp to the surface of a body of water a thoroughly successful selective flotation of 10 the oiled zinc sulfid is effected by surface tension.

Other modes of applying the principle of my invention may be employed instead of the one explained, change being made as 15 regards the process herein disclosed, provided the step or steps stated by any one of the following claims or the equivalent of such stated step or steps be employed.

I therefore particularly point out and distinctly claim as my invention:—

1. The process of concentrating ore, which consists in mixing together at a temperature of not less than 60° C. crushed ore, sufficient water to form a flowing pulp, sulfuric acid, 25 and a mineral oil in amount only sufficient to preferentially coat the desired sulfid particles of the ore; and thereafter presenting the pulp to the air and then to the surface of a liquid to cause a flotation of the oiled sulfid particles by surface tension.

2. The process of concentrating ore, which

consists in mixing together at a temperature of not less than 60° C. crushed ore, sufficient water to form a flowing pulp, an amount of sulfuric acid not over five per cent. of the ore by weight, and a mineral oil in amount only sufficient to preferentially coat the desired sulfid particles of the ore; and thereafter presenting the pulp to the air and then to the surface of a liquid to 35 cause a flotation of the oiled sulfid particles by surface tension.

3. The process of concentrating ore, which consists in mixing together at a temperature of not less than 60° C. crushed ore, sufficient 45 water to form a flowing pulp, an amount of sulfuric acid not over five per cent. of the ore by weight, and an amount of a petroleum oil of high boiling-point not over one per cent. of the ore by weight to preferentially 50 coat the desired sulfid particles of the ore; and thereafter presenting the pulp to the air and then to the surface of a liquid to cause a flotation of the oiled sulfid particles by 55 surface tension.

Signed by me, this 14th day of October, 1912.

WILLIAM SYDNEY STEVENS.

Attested by—

A. R. MINNER,  
M. G. BROWNE.